

Aug. 5, 1924.

1,504,139

W. F. R. PHILLIPS

DIAPHRAGM

Filed Sept. 16, 1921



W. F. R. Phillips  
INVENTOR.

BY

A. B. Foster  
ATTORNEY.

## UNITED STATES PATENT OFFICE.

WILLIAM F. R. PHILLIPS, OF WASHINGTON, DISTRICT OF COLUMBIA.

## DIAPHRAGM.

Application filed September 16, 1921. Serial No. 501,026.

*To all whom it may concern:*

Be it known that I, WILLIAM F. R. PHILLIPS, a citizen of the United States, residing at Washington, District of Columbia, 5 have invented new and useful Improvements in Diaphragms, of which the following is a specification.

This invention relates to a vibratory diaphragm for talking machines and other 10 sound reproducing instruments, the dominant resonating element of which is wood, that is, it is a diaphragm that is essentially a wooden diaphragm as to its dominant resonating properties and qualities, though 15 the diaphragm is not necessarily wholly of wood, but may consist of wood reinforced for the purpose of mechanical security with some membranous material, such as paper, parchment, celluloid, or other substance existing in or wrought into membranous condition.

The resonant properties and qualities of wood are well known and the use of wood as a resonator in musical instruments and 20 in talking machines is not claimed as new. Wooden diaphragms for talking instruments made of single continuous discs cut in the usual manners of cutting wood, that is quartered, bastard or transverse, (or cross 25 grain), are not satisfactory because of interferences in wave motion that result from the natural structure of wood as found in discs cut as described. One exception is to be noted, namely, if a disc were to be cut 30 cross grain and the section should contain the pith or marrow so located as to be at the center of the disc, such a disc would have a natural arrangement of the wood that will 35 not give rise to interferences in wave motion originating at the center of the disc. So far 40 as known no one has heretofore recognized this fact and it is therefore claimed as included in this invention, either unmodified or modified as hereinafter described. The 45 invention in the matter of wooden diaphragms for reproduction of sound in talking machines and instruments, and for short 50 hereinafter unless otherwise stated the term "diaphragm" only will be used, will be more readily understood by first stating briefly the structural peculiarities of wood and how 55 these peculiarities affect wave motion in diaphragms made of single pieces of wood cut in the usual planes in which timber is cut, namely, "quartered," (Fig. 7), "bastard"

(not illustrated), or "cross grain" (Fig. 8). Using the term in its common sense, wood is made up of two different parts, "spring wood" and "summer wood" arranged in concentric alternating rings, the "annual rings" 60 (Figs. 7 and 8) around the pith or marrow of the tree, easily seen as such in most woods cut transversely of the long axis of the tree. When cut lengthwise of the tree in the manner known as "quartered" the spring and the 65 summer woods appear as lines or bands of lighter and darker colors respectively. In "quartered" wood these bands or lines are quite regular in arrangement and appearance, and generally the spring wood is the 70 broader of the two. In "bastard" cuts the width of the lines or bands and their relations to each other and their directions are apparently very irregular, sometimes more spring wood sometimes more summer wood 75 being in evidence, according to the surface considered. Biologically the "spring wood" and the "summer wood" are alike. Physically the "summer wood" is the heavier or 80 denser and the "spring wood" the lighter or less dense. If there be any difference in the elasticity of the two it appears (so far as I am advised) not yet determined; biological considerations would seem to indicate that there is none. The densities being 85 known to be unequal, it follows that the velocity of wave motion in the two sorts is different, the velocity being in any medium proportional to the square root of the modulus of elasticity divided by the density 90 of the medium.

In a disc made of quartered wood, (for example like Fig. 7) in the direction of the grain, that is that of the lines or bands of the summer and spring woods, a wave 95 front would travel, be it in either the spring wood or the summer wood, in a medium relatively homogenous in structure and density, and its speed would be uniform. On the other hand, a wave traveling perpendicularly to the grain, would be passing through a medium alternately varying in density, and the wave would be subjected to retardations and reflections at every variation of density; its speed would not be 100 uniform, and its intensity or force would be decreased. A wave traveling diagonally across the grain would experience the same conditions, but the quantitative effect would be dependent on the angle of incidence 110

made with the bands of varying density. In a disc made of wood cut cross grain. (as for example Fig. 8) except in a disc made of such a section having the pith at its center, the same general conditions would obtain as in one cut of quartered wood. A disc made of bastard cut wood would be subject to the same general conditions, only in a more irregular and uncertain degree.

In discs of wood cut in the manners mentioned, the exception noted excepted, waves initiated at the center of such discs would travel not circularly, but more or less elliptically, or as ellipsoids. In sound reproducing diaphragms made of any of the discs above mentioned (except the one illustrated in Fig. 4) the major part of the wave would be reflected back to the center in a very complex form, which may be roughly said to be elliptoidal, with the long axis of the return wave at right angles to that of the original wave; altogether, the elliptoidal form of the original wave, the complex form of the return wave, the numerous asymmetrical reflections due to the asymmetry of the grain to the center, give rise to many interferences in wooden diaphragms of single pieces of wood, the single exception above noted excepted.

Briefly this is why ordinarily the forms in which wood is cut, are unsuited to be worked into single piece sound reproducing diaphragms, the exception above noted excepted.

Fig. 1 is a cross section of a simple form of diaphragm made of wood, and having a paper or other membranous facing and backing, either one of which can be omitted. In this figure, the tapering thickness is exaggerated. Fig. 2 is a simple form of a built-up diaphragm, composed of four wooden sectors, cut quartered, the grain running at right angles to the central radius this being the axis of symmetry of each sector. Fig. 3, shows a similarly constructed diaphragm, with the grain parallel to the central radius of each sector. Fig. 4 shows a cross cut diaphragm, made of one piece, the pith of the tree at the center of the diaphragm. Fig. 5, shows a built-up diaphragm simulating that shown in Fig. 4 through the medium of the central pin or stylus holder. Fig. 6, shows one mode of mounting the diagrams on the sound box. Figs. 7 and 8 show respectively discs of quartered wood and cross cut (ordinary or non-central) wood. These latter make unsatisfactory diaphragms for the reasons above set forth.

The diaphragm is a thin, circular disc, wholly of wood or formed of wood and membrane, such as paper, parchment, celluloid, or other material already alluded to. The diaphragm is shown diagrammatically the wooden portion thereof being in perpen-

dicular medial section in Fig. 1, indicated by the numeral (4). The small central projection (5) is a wooden peg or pin, for attaching the actuating end of the needle lever to the diaphragm, and is designated the "union." The thickness of the diaphragm varies somewhat according to its diameter and the manner of the construction of the diaphragm itself. Generally the thickness may be about 1/32 inch at its center and not substantially more than 1/100 inch at the periphery. Wood diaphragms having a maximum thickness of less than 1/64 of an inch, seem to lose the peculiar tonal properties that make wood desirable as a reproducing diaphragm.

In practice, diaphragms appear to give better results if thicker in the center than at the periphery. In the diaphragms herein described the central part is always the thickest and the periphery the thinnest. Between these two parts, the thickness diminishes either gradually and uniformly, or uniformly and more or less gradually, producing either an inclined plane, a convex, or a concave surface, or surfaces, or any desired combination of them. No one shape seems to be better than another, but a plano-inclined surface as contra a plano-concave or plano-convex, is contemplated. Thus the preferred form of construction of the diaphragm is that of a very flat cone.

The wood of which the diaphragm may be made, in whole or in part, may be of any kind, but soft woods, and particularly soft and brittle woods, such as white pine, cedar, balsa and "old field pine," (a short leaf pine which is cheap and abundant, and commonly used for making light packing boxes), also called "loblolly pine" in some localities have been found to give particularly good results. These woods are generally soft, quite brittle, and are quite generally available. They are relatively homogeneous in structure, the variation in density between the softer part and the harder part of the annual rings is low, as compared with other kinds of wood, and they possess excellent tonal qualities.

Soft, but relatively tough woods, such as spruce, do not appear to possess the resonant qualities of the soft and brittle woods, and are not well suited for sound box diaphragms.

A wood diaphragm of the thinness and of the kinds of wood described may be easily damaged, split or broken, by careless handling, particularly by splitting in the direction of the grain of the wood. Such accidents may be minimized without impairing apparently the resonant qualities of the diaphragm by facing one or both of its surfaces with some thin fibrous paper, such as "onion skin" paper, or by a thin film of celluloid or parchment, or other membranous

material of equivalent thickness or tenacity, as shown in Fig. 1. Also wood being to a limited degree hygroscopic, and its resonant quality being impaired by an excess of absorbed moisture, facing the diaphragm on one or both sides inhibits undue absorption of atmospheric moisture. Furthermore, efficient waterproofing may be applied to the paper or other membrane without impairing the resonant quality of the wood, something difficult to do when the waterproofing is applied direct to the wood. When a membrane (paper or the like) is not applied to the front side of the wooden diaphragm, this may be given a light coating of a suitable varnish, and it is preferred that this be applied superficially, as much as possible, since an impregnation of the wood with varnish, or the like, is injurious to its tonal qualities.

The diaphragms to be hereinafter described in more detail, will therefore be faced on one or both sides for the purposes indicated, and when so faced the membranous facing becomes an integral part of the diaphragm and continues it in extent, forming an annular ring of membranous material of determinate width, around the wooden portion. The diaphragm is secured to its support through this membranous ring.

The diaphragms shown in Figs. 2, 3, and 5 are each made of four or more sectors cut and joined by glue or other cement so as to give an approximate concentric arrangement of the grain within the disc area. This symmetrical ordering of the grain obtained by this arrangement, insures far more uniformity of resistance to pressure in all diameters and consequently more uniformity of vibrating movement of the diaphragm. Obviously the uniformity approaches the limit of absoluteness as the number of the sectors is increased. However, in practice no appreciable improvement is noticed beyond six or eight or ten sectors. Diaphragms of this type reproduce satisfactorily all kinds of phonographic records seemingly with perfect fidelity to the original as recorded on the phonograph disc.

The diaphragm shown in Fig. 4 is made by cutting the wood transversely as in Fig. 8, but the section is cut from the heart region of the wood and has as its own center the natural center of the wood, therefore as perfect uniformity of grain is thus obtained as is practicable.

In wood diaphragms built up of sectors, the invention is not restricted to the use of a particular number of such sectors. In those shown in Figs. 2, 3 and 5, the sectors are attached to each other, and to the union or pin 5 preferably by a suitable glue or cement. Ordinary carpenter's glue can be employed. It will be clear that the greater

number of sectors, the more closely absolutely the finished diaphragm should approach absolute uniformity if the cement or glue used in attaching each sector to its neighbor, were absolutely homogeneous with the wood. However, the two are not homogeneous with each other, and ordinarily the use of more than eight or ten sectors is not advantageous. Obviously, no excessive amounts of glue are to be used, since as above stated, it is not desired to impregnate the wood with any foreign substance.

The diaphragms shown, Figs. 2, 3, 4 and 5 are of wood faced on one or both surfaces with paper, celluloid, or parchment, or other membranous material.

Fig. 6 shows the relation between the wooden portion and the membranous portion of the diaphragm, seen either from the front or back. In this figure, 5 is the union or connecting pin, 13 is the wooden disc, 14 is the inner margin of the funnel of the sound box, 16 is its outer margin, the membranous portion of the diaphragm uncovered by the wooden portion extends laterally from 13 to 16.

Referring again to Fig. 4 of the drawing, if a cross-grain section of wood that includes the pith or marrow be taken and a disc cut from it so as to have the pith as the center, it will be seen that the spring and summer woods are substantially symmetrically disposed about the center. If pains be taken in selecting the wood the degree of symmetry can be brought very near absolute. A wave initiated at the center of a carefully selected disc will be subject to retardations and reflections due to the alternate variations in density of the spring and summer woods. However these retardations and reflections will be symmetrical in all radii, and therefore interferences will not occur. The wave will advance from and return to the center as little interfered with in form, as if in a homogeneous medium. A diaphragm fashioned with respect to the grain and pith as above described and shown in Fig. 4, is original so far as relates to diaphragms for sound reproducing machines. The other diaphragms shown in Figs. 2, 3, and 5, are approximations of this symmetry.

The fundamental principle involved in making a workable wooden diaphragm may be stated as radial symmetry in the disposition of the grain.

By radial symmetry as herein applied to wooden diaphragms is meant any arrangement of the grain of the wood about the center of the diaphragm whereby the grain of the wood will be so balanced with respect to the center of the diaphragm that any and every radius shall hold. (within limits indicated herein) with respect to any and every other radius with which it may be compared, the same relation to the grain

of the wood. That is, if one radius is perpendicular to the grain or to the cord of the arc of the concentric rings, every other radius is and this constitutes the preferred construction.

I propose to construct diaphragms of sectors cut from "quartered" wood, and to arrange them either so that the grain shall be concentrically disposed around the center, as in Fig. 2. The specification of diaphragms made of 4 to 10 sectors, is not to be understood as limiting the number, but I may avail myself of whatever number may be deemed most suitable either with respect to the size of the diaphragm or the quality of the wood used, or both.

Experiments have demonstrated that in diaphragms in which the wood, is arranged as above described, wave motions initiated at the center will be propagated more or less circularly and symmetrically and will be free from the interferences inherent in wooden diaphragms constructed of single pieces, the exception above noted excepted.

A diaphragm for talking machines to be commercially valuable, should be capable of reproducing most of the phonographic records on the market. To meet this requirement the diaphragm must have the elastic qualities of the diaphragms making the record or for which the record is made. The effective vibrating surface of diaphragms in use, is between 1-3/4 and 2 inches. A wooden diaphragm constructed of sectors as above described, the wood used being white pine, and having an effective diameter of 2 inches, to be capable of reproducing the record as perfectly as recorded is found to weigh less than 40 milligrams, the best results being obtained with one in which the weight of the wood as finally finished was 35 milligrams. A wooden disc made up of eight white pine sectors 2-1/4 inches in diameter, the size necessary to secure the periphery to the sound box rim, which weighed 37 milligrams, was found to be about 1/64 inch thick at the center and to taper to less than 1/100 at the periphery. Such a disc is too fragile for the usage to which a talking machine diaphragm is subjected. However, a diaphragm of this description can be made strong enough to withstand the ordinary usage to which subjected by reinforcing it with some tough but light membranous material, such as onion skin or other thin, tough paper, celluloid, vegetable parchment, or other similar light and tough membranous material. In practice I have used thin onion skin or similar paper impregnated with thin celluloid varnish. Such a membrane is very light, strong and thin, being not over .002 of an inch thick. When a wood diaphragm as described is reinforced by being mounted on a membrane made of such paper, it is practicable to dispense with

so much of the wood as might extend upon the rim of the sound box, replacing it by extending the membrane thereon. In actual practice better results have been obtained by still further reducing the diameter of the wooden disc. A wooden disc of 1-3/4 inches mounted on a membrane of paper and varnish as above described, thus giving in a 2 inch diaphragm a membranous margin of 1/8 inch inside the rim of the sound box is a very satisfactory diaphragm. I therefore propose to so mount any, and all, of the wooden diaphragms herein described. The above dimensions are given by way of illustration only. The woods of which I propose to make these diaphragms may be of any kind, but in practice, I prefer white pine, and have obtained very satisfactory tonal results from it. Next to white pine, I have found selected pieces of loblolly or old field pine very satisfactory. Cedar, yellow pine and balsa have also given good results.

Comparing wood with membrane such as paper, parchment, or celluloid, for equal weights, the membrane will be found the stronger in most directions. Now experiment shows that as already stated wood has the most suitable tonal qualities as a general reproducing medium; experiment shows also that membranes such as mentioned are deficient in tonal qualities. A paper combination of wood and of membrane, therefore, seems to be the desideratum. In the diaphragm shown in Fig. 7, this end is sought to be obtained.

It appears advisable in most cases, not to employ excessive amounts of paper or membranous materials. One thickness or at most two of such paper as "onion skin" (say on the outside) with the other side of the wood uncovered (or preferably coated with an extremely thin coat of a waterproofing agent, such as shellac), gives better results than a thickness of paper on both surfaces. A plurality of thickness of paper, on either one or both sides of the wooden disc seems to materially reduce the tonal quality of the reproduction.

The preferred construction is to employ the smallest amount of wood necessary to give the optimum tonal quality. An excess of wood seems to slow down the vibrations and hence to reduce the volume of sound. Several thicknesses of paper have a like effect, to some extent, and also will reduce the tonal quality to a greater degree.

I claim:

1. A diaphragm comprising a wooden disc constructed of not less than four wooden sectors, the sectors equal in size and the grain of the wood of every sector perpendicular to the axis of symmetry of the sector; this wooden disc being attached to and reinforced by a thin membranous disc, of

material of approximately the thickness of onion skin paper, such membranous disc being of a greater diameter than the wooden disc, whereby the completed diaphragm 5 shows a central wooden disc surrounded by a membranous margin of a determinate width.

2. A diaphragm built up of not less than four sectors of the same size, the grain of the 10 wood being symmetrically arranged in each of said sectors, and said sectors being joined to each other by a cementing material

and having the grain of the wood approximately at right angles to the radius of symmetry of the sector as hereinbefore described. 15

3. A diaphragm comprising at least four wooden sectors having the grain approximately radially symmetrically disposed around the center of the diaphragm in such manner that the grain is substantially perpendicular in each sector to the axis of symmetry of the sector. 20

In testimony whereof I affix my signature.  
WILLIAM F. R. PHILLIPS.